

## UNITED STATES PATENT OFFICE

2,099,782

## TEXTILE PRINTING PROCESS AND PRINTING PASTE THEREFOR

Ernst Weiss, Wattwil, Switzerland, assignor to  
Heberlein Patent Corporation, New York, N. Y.,  
a corporation of New York

No Drawing. Application July 9, 1935, Serial  
No. 30,519. In Germany and Great Britain  
July 26, 1934

## 4 Claims. (Cl. 8—20)

This invention relates to a textile printing process and a printing-paste therefor. It is more particularly directed to a process for printing cotton or other cellulose-containing fabric with a paste containing a thiocyanate.

The action of calcium thiocyanate for printing on cotton and rayons is known. The thiocyanate has a parchmentizing effect on the fabric under the simultaneous action of heat and moisture so that where the thiocyanate acts on the fabric it produces greater transparency. Great difficulty has been experienced in attempts to use this process because of the fact that the thickened calcium thiocyanate printing mass must be maintained in heated condition during use and the heat must be suitably regulated to prevent the mass from stiffening. At ordinary room temperature, say 65° F. or somewhat above, the printing masses heretofore employed stiffened or 15 jelled and were not suitable for printing.

I have now found in accordance with my invention that the jelling of the combination of a thiocyanate, water and a thickener which would ordinarily act on one another to cause a jelly to form at low temperatures, can be avoided by the presence of an aliphatic aldehyde such as formaldehyde. By the use of the combination just mentioned a printing-paste which can be printed cold without difficulty is obtained. The mass has 20 a better viscosity for penetration of the fibers of the fabric than the heated printing-paste heretofore employed. It accordingly better penetrates the fibers. I have found also that by addition of formaldehyde to this printing mass that the swelling action of the calcium thiocyanate is 25 increased.

As thickeners I have found that both, starch and cellulose which are well-known as thickeners may be employed. Other thickeners can also be 30 used for example cellulose-derivatives. I prefer to employ reprecipitated cellulose as for instance viscose waste and have found such reprecipitated cellulose exceptionally suitable as a thickening agent.

45 My process can be applied to all kinds of cellulose-containing fabrics such as flat fabrics, knit goods, braided goods, embroideries and the like. Fabrics may be employed which contain yarns 50 of different fiber materials as for instance mixed fabrics or fabrics made from mixed yarns. Of the artificial fiber materials those of reprecipitated cellulose and those produced from cellulose esters are suitable. The expression "cellulose-containing fabrics" is intended to cover such fab-

rics of artificial or natural fibers or mixtures thereof.

The fabrics prior to the printing with the thiocyanate printing-paste may be pretreated in any desired manner. For example they may be 5 boiled, half- or full-bleached or mercerized.

After the printing of my improved paste the fabrics are dried and thereupon I ordinarily develop the effect in the case of cotton or similar natural fiber by steaming or passing through a 10 concentrated hot salt solution such as calcium chloride at a temperature above 100° C. After this treatment the fabrics are washed and dried. Artificial silk fabrics as a rule do not require any 15 steaming or calcium chloride process but can be washed directly after the drying of the printing.

For certain kinds of fabrics, viz. cotton-mouseline, -satin, -voile, subsequent mercerization can be applied under tensioning. Intensification of the fancy printed effects can be obtained by 20 after-treatment of the loose fabric with swelling agents which have a shrinking effect. My present process can be combined as desired with different kinds of dyeing and color printing either before or after the printing with calcium thiocyanate. 25

The following are examples of the process. They are to be regarded as illustrative and the invention is not restricted thereto.

## Examples

30

1. Bleached, mercerized, cotton mouseline fabric is printed at about 18° C. with the following mass:

|                                                                                 | Grams | 35 |
|---------------------------------------------------------------------------------|-------|----|
| Calcium thiocyanate crystallized                                                | 710   |    |
| Water                                                                           | 106   |    |
| Viscose waste                                                                   | 22    |    |
| Formaldehyde concentrated technical (industrial) formaldehyde content about 40% | 40    |    |
|                                                                                 | 162   |    |
|                                                                                 | 1000  |    |

The fabric is well dried in the loft at about 45 80° C. and thereupon immediately passed through a developing bath of the following composition:

|                              | Parts by weight |
|------------------------------|-----------------|
| Calcium chloride, granulated | 3               |
| Water                        | 2 50            |

The temperature of this bath is kept at 115-120° C. The time of action is about 15 seconds; after this passage the fabric is washed cold, centrifuged, finished and dried. 55

|                                                                                      |       |
|--------------------------------------------------------------------------------------|-------|
| 2. A viscose fabric is printed at about 18° C. with the following mass:              | Grams |
| Calcium thiocyanate crystallized.....                                                | 650   |
| 5 Water.....                                                                         | 170   |
| Viscose waste.....                                                                   | 18    |
| Formaldehyde concentrated technical (industrial) formaldehyde content about 40%..... | 162   |
| 10                                                                                   | 1000  |

After the drying of the printing, the fabric is immediately washed cold, centrifuged and the drying is completed.

- 15 3. A mousseline fabric is printed in accordance with the instructions of Example 1, with calcium thiocyanate, developed in a calcium chloride bath at about 115°-120° C. and washed. Thereupon it is placed in loose condition in a sodium hydroxide solution of 30° Bé. at room temperature for 3 minutes, soured with sulphuric acid of 2° Bé. and the washing is completed. This action results in the fabric shrinking and becoming more dense.
- 20 4. A viscose voile fabric is printed with the following mass:

|                                                   |      |       |
|---------------------------------------------------|------|-------|
| Calcium thiocyanate crystallized.....             | 684  | Grams |
| Water.....                                        | 105  |       |
| 30 Formaldehyde concentrated technical (40%)..... | 158  |       |
| Wheat starch.....                                 | 53   |       |
|                                                   | 1000 |       |

- 35 After the mass is printed, the fabric is dried, rinsed with cold water and then dried on a tenter frame.

5. A cotton mousseline fabric as used in Example 1 is printed with the following mass:

|                                                |      |       |
|------------------------------------------------|------|-------|
| 40 Calcium thiocyanate crystallized.....       | 700  | Grams |
| Water.....                                     | 100  |       |
| Acetate silk waste.....                        | 30   |       |
| Formaldehyde concentrated technical (40%)..... | 170  |       |
|                                                | 1000 |       |

The further treatment is done as in Example 1. The viscose waste mentioned in the above examples consists of viscose silk cut in short staples. Other reprecipitated cellulose may be em-

ployed if desired. Other salts or agents than calcium chloride may be employed in the development bath. Calcium chloride is representative of an inexpensive compound which will raise the temperature of the bath to about 115-120° C. and effect the desired development.

The result of the above printing is to produce a fabric having relatively transparent portions on a less transparent background. These effects as noted above may be combined with other effects produced by mercerization, shrinkage, etc.

The expression "room temperature" as employed in the claims and elsewhere herein is intended to designate a temperature of about 18° C. (about 65° F.) or temperatures somewhat above or below that point.

I claim:

1. A process for printing cellulosic fabrics or the like which comprises combining calcium thiocyanate, water and a thickener consisting of re-precipitated cellulose which would ordinarily act on one another to produce a jelly at room temperature and also combining therewith a sufficient quantity of formaldehyde to oppose such jellying action to produce a paste for printing on cellulose fabrics and printing such paste on a cellulose fabric at room temperature.

2. A step in the process of printing cellulosic fabrics which comprises treating a cellulose fabric at low temperature with a combination of a thiocyanate, water and a thickener which would ordinarily act on one another to produce a jelly at room temperature, and formaldehyde to oppose such jellying.

3. A process for printing which comprises printing a cotton fabric at low temperature with a combination of calcium thiocyanate, water and a reprecipitated cellulose as a thickener which would ordinarily act on one another to produce a jelly at room temperature, in the presence of formaldehyde to oppose such jellying, and developing such printing above 100° C. in a salt bath containing sufficient salt to raise the boiling temperature of the bath above said last mentioned temperature.

4. A printing-paste containing calcium thiocyanate, water and viscose waste which would ordinarily act on one another to produce a jelly at room temperature and formaldehyde to prevent jellying of paste at such temperature.

ERNST WEISS.